

1

3,047,390

METHOD FOR OPTICAL BLEACHING  
COATED PAPERS

Willem Karel Koerber and Ferdinand Leonard Schouteden, Wilrijk-Antwerp, Belgium, assignors to Gevaert Photo-Producten N.V., Mortsel, Belgium, a company of Belgium

No Drawing. Filed June 2, 1958, Ser. No. 739,211  
Claims priority, application Netherlands June 6, 1957  
9 Claims. (Cl. 96—82)

The present invention relates to a process for whitening the surface color of papers provided with one or more surface coatings the composing elements of which are not able to strongly bind optical bleaching agents, and more particularly relates to a process for brightening the white areas in photographic images whereby the wandering of optical bleaching agents out of the photographic layers is inhibited.

It is generally known that the reflecting power of the paper surface can considerably be increased by applying a surface coating containing filling substances with a high degree of whiteness. Examples of such filling substances are i.a. titanous dioxide, barium sulphate, zinc sulphide, calcium carbonate and silicon dioxide. In this way, the surface color of the paper can be whitened to a certain extent, but not completely. If, however, a paper is concerned where this surface coating contains besides the white pigments products which are slightly colored or which are colored during the further treatments or during the storage of the paper or where on this surface coating still one or more other layers are coated which contain such products, the brightening effect obtained by applying the reflecting surface coating is nullified wholly or partially. Thus it is seen for instance that when a baryta-coated paper support is coated with a photographic emulsion, the surface color of the photographic paper is not completely white so that even the whitest areas in a photographic image obtained upon such a support still absorb a considerable amount of light. This coloration depends on various factors such as the reflecting power of the used paper, the quality of the gelatin applied as binding agent for the photographic layers and the kind and the amount of compounds such as e.g. sensitizing dyestuffs added to the photographic layers during the manufacture of the light-sensitive element. This coloration can also be caused by colored decomposition products which are formed during the development and further treatments of the photographic element in the photographic layers or are absorbed by these layers from the baths wherein they were formed. Since the cellulose fibers wherefrom the paper is composed, as well as the gelatin used as binding agent for the photographic layers and the decomposition products which are formed during the processing absorb the light particularly in the range of the short wave-lengths, the photographic paper shows in most cases a slight yellow tinge.

It has been proposed to eliminate this defect by adding to the paper support, to a surface coating and/or to another superposed layer, dyestuffs or pigments which absorb in the range of the long wave-lengths, so that the spectral partition of the reflected visible light is equal to that of the incident visible light and the paper shows a neutral tone. Thus, it is known to add organic light-fast blue dyestuffs to a baryta-coating which is applied to a paper support destined for receiving a photographic emulsion layer.

By application of this process, the incident visible light is not completely reflected but partly absorbed by the yellow paper and partly by the blue dyestuff or the blue pigment. Even in the most favorable cases where only an extremely small amount of dyestuff or pigment is re-

2

quired, such as for instance for the manufacture of a photographic paper starting from a baryta-coated paper of good quality, from a little colored gelatin and from sensitizing dyestuffs which during the processing can easily be removed from the photographic layers, the whitest areas in the photographic image will not completely reflect the visible light.

According to a more recent process, substantially colorless blue-fluorescing ultraviolet-absorbing compounds are added during the manufacture to the paper or to one or more surface coatings e.g. compounds absorbing ultraviolet radiation of between about 3000 Angstrom units and 4000 Angstrom units and emitting fluorescent light of between about 4000 Angstrom units and 5500 Angstrom units. These compounds can be added during the manufacture of a photographic paper for instance to the paper support, to the layer wherein the photographic image is formed (for instance the silver halide emulsion layer) or to a layer therebetween (for instance a baryta-coating). The photographic element can also be treated with a solution of such compounds during the processing.

The spectral partition of the reflected visible light is equalized by the use of these optical bleaching agents to that of the incident visible light by conversion of a part of the incident ultra-violet rays to which the human eye is not sensitive into the blue light absorbed by the paper. The reflected light is now completely neutral, without loss of a part of the visible incident light. By applying this method in the manufacture of photographic paper, it is not only possible to obtain a neutral image tone together with a strong reflecting power of the white areas in the photographic image, but moreover photographic images to be viewed by reflection can be manufactured which reflect more visible light than they properly receive, i.e. when an excess of optical bleaching agent is used so that more ultra-violet light is converted into blue light than is necessary to correct the yellowness of the photographic paper. In this way, it is possible to change the image-tone to a colder, i.e. a more bluish tone.

In connection with the above described process, according to which an optical bleaching agent is added to the paper itself and/or to the baryta-coating and/or to the emulsion layer, it is to be noted that by the addition of the optical bleaching agent to the paper alone, no sufficient brightening of the images is obtained, since the whitening effect is annulled for a great part by the superposed baryta-coating which is present in most of the photographic papers.

It is evident that the practical result, which can be attained when applying the above-mentioned process, 50 depends on the amount of optical bleaching agent which is still present in the completely finished paper. Consequently, it has been tried to prevent that the optical bleaching agents should be removed wholly or partially 55 from the layers of the photographic element for instance when treating the photographic elements in the usual treating baths.

None of the different propositions to counteract the wandering of the optical bleaching agents out of the emulsion and/or the baryta-coating has hitherto been 60 found effective in this respect.

Summarizing, the great difficulty in finding an effective solution for this problem mainly results from the fact that the optical bleaching agents are not or at least insufficiently adsorbed on elements, such as gelatin and baryta of which the usual surface-coatings applied to the paper are composed.

It is therefore an object of the present invention to provide a method for increasing the whiteness of the surface 70 of a paper provided with at least one surface coating whereby the wandering of the optical bleaching agents out of the layers wherein they were incorporated is inhibited.

It is a further object of the present invention to provide a method for increasing the whiteness of photographic papers. Still further objects will appear in the following description and examples.

It has now been found that the wandering of optical bleaching agents out of the layers in which they were incorporated can be inhibited completely by treating finely divided water-insoluble macromolecular products with a solution or a dispersion of an optical bleaching agent which possesses a pronounced substantivity to the macromolecular product used and by adding the fluorescing mass obtained to one or more surface coatings. Thus, in the manufacture of a photographic paper the fluorescing mass can be incorporated into a layer between the paper-support and the layer wherein the photographic image is formed or into the latter layer itself. Macromolecular products which in finely divided state are suitable for carrying out the method according to the present invention, are i.a.: cellulose, polyesters, polyamides and ureaformaldehyde resins. As distinct from the generally adopted tendency, which consists in using polymers with high degree of polymerization for most of the applications, those polymers having a low degree of polymerization are to be preferred among the synthetic polymers for carrying out the process according to the present invention since contrary to the high polymeric products they can be divided very finely and in this way can bind relatively more bleaching agent.

Suitable polyesters for carrying out the process according to the present invention are for instance the oligomers of aromatic polyesters which can be prepared in a simple way by re-esterifying the dimethyl ester of an aromatic acid with a lower diol in the presence of a catalyst which mainly influences the re-esterification and to a less extent the polycondensation. For further elucidation, we give hereinafter some examples relating to the preparation of some oligomers of the polyester type which can be applied for carrying out the process according to the present invention.

#### PREPARATION 1

100 g. of dimethylterephthalate, 75 cm.<sup>3</sup> of ethylene-glycol (molar proportion 1:2.63) and 0.015 g. of zinc acetate are heated for 3 hours in such a way that the liberated methanol (about 40 cm.<sup>3</sup>) is slowly distilled over. When no methanol distills over anymore, temperature is raised to 180-190° C. and slowly increased until about 30 cm.<sup>3</sup> of glycol has distilled over. The reaction mixture is crushed after cooling and as the case may be, ground under the addition of a certain amount of water.

#### PREPARATION 2

100 g. of a mixture consisting of equal parts of iso- and terephthalic acid dimethylester, 75 cm.<sup>3</sup> of glycol and 0.030 g. of zinc monomethyl terephthalate are heated for 3 hours so that the liberated methanol slowly distills over. When no methanol distills over anymore, the temperature is raised to 180-190° C. and slowly increased until 38 cm.<sup>3</sup> of glycol has distilled over. After cooling, the reaction mixture is crushed and as the case may be, ground under addition of a certain amount of water.

#### PREPARATION 3

50 g. of dimethylisophthalate, 50 g. of dimethyl-p-carboxyphenyl-sulphone, 60 cm.<sup>3</sup> of glycol and 0.020 g. of zinc acetate are heated for 3 hours, so that the liberated methanol distills over slowly. When no methanol distills over anymore, the temperature is raised to 200° C. and maintained until about 30 cm.<sup>3</sup> of glycol has distilled over. After cooling, the reaction mixture is crushed and as the case may be, ground under addition of a certain amount of water.

A polyamide which is suitable for carrying out the method according to the present invention can be prepared as follows:

#### PREPARATION 4

20 g. of caprolactam and 0.05 g. of carbonate-free sodium hydroxide are heated for about 10 minutes at 95° C. whilst pure nitrogen is bubbled through. Thereafter, heating is continued for another 20 minutes at 230° C. and then the reaction mixture whilst strongly stirring is poured out into 1½ l. of water, sucked off and thoroughly washed with warm water.

Suitable optical bleaching agents for carrying out the process of the present invention are described i.a. in Phot. Korrespondenz, 94 (1958), p. 5.

For carrying out the process according to the present invention, a certain amount of the finely divided macromolecular product is dispersed in water. To this suspension is added a solution of the optical bleaching agent involved. If the optical bleaching agent is not or not sufficiently soluble, it can be added in dispersed form to the suspension. The treatment of the macromolecular product with the optical bleaching agent is preferably carried out at a temperature between 50 and 100° C. and is continued until no more fluorescing substance is bound. After sucking off, a strongly fluorescing paste is thus obtained which strongly retains the fluorescing substance and which can be added to the coating composition which is to be applied to a paper support. Thus the fluorescing mass can for instance be added to a baryta-composition which is spread upon a paper whereon a photographic emulsion is to be coated. The fluorescing paste can, as the case may be, be incorporated in a photographic emulsion itself, in which case very favorable results can be attained by using as macromolecular product an ureaformaldehyde resin such as described in the Belgian specification 451,470 and which i.a. also comprises condensation products with a characteristically low degree of polymerization.

The wandering of the optical bleaching agent out of the layer, wherein it was applied, is practically completely excluded by applying the method according to the present invention, so that the exposed photographic element after complete processing, which even may comprise a protracted rinsing, yields a photographic image wherein the white areas are strongly brightened.

The method according to the present invention can be applied for brightening the white areas in usual photographic black-and-white and colored images as well as for whitening the surface color of any other surface-coated paper such as for instance papers on which a positive photographic image is formed by applying the silver halide diffusion transfer process, or papers on which an image is printed by means of an hectographic process.

The present invention is further illustrated in the following examples without limiting, however, the scope thereof. The formula of some of the optical bleaching agents used in the examples, are shown in the accompanying drawings.

#### Example 1

1 kg. of the polyester paste, obtained according to Preparation 1 is dispersed in 1500 cm.<sup>3</sup> of a 5% aqueous solution of sodium sulphate together with 10 g. of  $\alpha,\beta$ -di(5-methylbenzimidazyl-2)-ethylene (cf. formula 1). By strongly stirring, the whole mass is kept in suspension for 30 minutes at a temperature of 80-90° C. After this treatment, the fluorescing mass is sucked off and the strongly fluorescing paste thus obtained is added to a baryta composition which is spread on a paper to be coated with one or more photographic emulsion layers. The whiteness of the surface color of the photographic paper thus treated is not lost on rinsing and the photographic element yields after exposure and complete finishing a photographic image wherein the white areas are strongly brightened.

A similar result is attained when on carrying out the process of the present example, the  $\alpha,\beta$ -di(5-methylbenzimidazyl-2)-ethylene is replaced by a same amount of 1,3-dioxo - 2 - butyl - 6-acetylamo-1,2,3H-benz[de]isophthalate.

## 5

quinoline (cf. Formula 2), or  $\alpha,\beta$ -di-(benzimidazyl-2)-ethylene (cf. Formula 11).

## Example 2

1 kg. of the polyester paste obtained according to Preparation 2 is dispersed in 1500 cm.<sup>3</sup> of water together with 10 g. of  $\alpha,\beta$ -di(5-methylbenzimidazyl-2)-ethylene (cf. Formula 1). By strongly stirring, the whole mass is kept in suspension for 30 minutes at a temperature of 60° C. After this treatment, the fluorescing mass is sucked off and the strongly fluorescing paste thus obtained is added to a baryta composition which is spread on a paper. The surface color is clearly white and is not modified when the paper is rinsed with water for a longer time.

A similar result is attained when on carrying out the process of the present example, the  $\alpha,\beta$ -di(5-methylbenzimidazyl-2)-ethylene is replaced by a same amount of 1,3 - dioxo - 2 - butyl - 6 - acetylamino-1,2,3H-benz[de]isoquinoline] (cf. Formula 2) or  $\alpha,\beta$ -di(5-methylbenzoxazolyl-2)-ethylene (cf. Formula 12).

## Example 3

1 kg. of the polyester paste obtained according to preparation 3 is dispersed in 1500 cm.<sup>3</sup> of a 5% aqueous solution of sodium sulphate together with 10 g. of  $\alpha,\beta$ -di(5-methylbenzimidazyl-2)-ethylene (cf. Formula 1). By strongly stirring, the whole mass is kept in suspension for 30 minutes at a temperature of 90° C. After this treatment the fluorescing mass is sucked off and treated as indicated in Example 1.

A similar result is attained when on carrying out the process of the present example, the  $\alpha,\beta$ -di(5-methylbenzimidazyl-2)-ethylene (cf. Formula 1) is replaced by a same quantity of 1,3-dioxo-2-butyl-6-acetylamino-1,2,3H-benz[de]isoquinoline (cf. Formula 2),  $\alpha,\beta$ -di(benzimidazyl-2)-ethylene (cf. Formula 11) or  $\alpha,\beta$ -di(5-methylbenzoxazolyl-2)-ethylene (cf. Formula 12).

## Example 4

1 kg. of the polyamide paste obtained according to the Preparation 4 is suspended in 1500 cm.<sup>3</sup> of a 5% aqueous solution of sodium sulphate together with 10 g. of 4,4'-bis(2 - hydroxy - 4-phenylamino-1,3,5-triazyl-6)-diaminostilbene-2,2'-disulphonic acid disodium salt (cf. Formula 3). By strongly stirring the whole mass is kept in suspension for 30 minutes at a temperature of 80-90° C. After this treatment the fluorescing mass is sucked off and treated as indicated in Example 1.

A similar result is attained when on carrying out the process of the present example, the 4,4'-bis(2-hydroxy-4-phenylamino - 1,3,5 - triazyl - 6)-diaminostilbene-2,2'-disulphonic acid disodium salt is replaced by the same amount of  $\alpha,\beta$ -di(5-methylbenzimidazyl-2)-ethylene (cf. Formula 1) or  $\alpha,\beta$ -di(5-methylbenzoxazolyl-2)-ethylene (cf. Formula 12).

## Example 5

1 kg. ground cellulose is dispersed in 1000 cm.<sup>3</sup> of water. To this suspension are added 400 cm.<sup>3</sup> of a 1% aqueous solution of the compound 4,4'-bis(2-hydroxy-4-phenylamino - 1,3,5 - triazyl - 6)-diaminostilbene-2,2'-disulphonic acid disodium salt (cf. Formula 3). By strongly stirring, the whole mass is kept in suspension at a temperature of 50-100° C. until no more fluorescing substance is bound by the cellulose. After this treatment the fluorescing mass is sucked off and the thus obtained strongly fluorescing paste is added to a baryta composition which is spread upon a paper whereon one or more photographic silver halide emulsion layers are to be coated. The whiteness of the surface color of the photographic paper thus treated is not lost on rinsing and the photographic element yields after exposure and complete finishing a photographic image wherein the light parts are strongly brightened.

A similar result is attained when in the execution of the process of the present example, the 4,4'-bis(2-hydroxy-

## 6

4 - phenylamino - 1,3,5 - triazyl-6)-diaminostilbene-2,2'-disulphonic acid disodium salt is replaced by a same amount of 4,4' - bis(2 - amino - 4-hydroxyethylamino-1,3,5 - triazyl - 6) - diaminostilbene - 2,2' - disulphonic acid disodium salt (cf. Formula 4), 4,4'-diaminostilbene-2,2' - disulphonic acid (Formula 5), 4,4'-bis[2,4-di(n-butoxypropylamino) - 1,3,5 - triazyl - 6] - diaminostilbene - 2,2'-disulphonic acid (Formula 6), 4,4'-bis[2,4-di(isooctylphenoxyethoxypropylamino) - 1,3,5 - triazyl-6] - diaminostilbene-2,2'-disulphonic acid (Formula 7), 4,4' - di(phenylureido) - stilbene - 2,2' - disulphonic acid disodium salt (Formula 8).

## Example 6

15 1 kg. of ground cellulose is dispersed in 1000 cm.<sup>3</sup> of water. To this suspension are added 400 cm.<sup>3</sup> of a 1% ethanol solution of the compound 1,3-dioxo-2-butyl-6-acetylamino-1,2,3H-benz[de]isoquinoline (cf. Formula 2). By strongly stirring, the whole mass is kept in suspension at a temperature of 50-100° C. until no more fluorescing substance is bound by the cellulose. After this treatment, the fluorescing mass is sucked off and further treated as indicated in Example 5.

A similar result is attained when on carrying out the process of the present example, the 1,3-dioxo-2-butyl-6-acetylamino-1,2,3H-benz[de]isoquinoline is replaced by a same quantity of 1,3-diphenyl-5(p-iodophenyl)-pyrazoline (Formula 9).

## Example 7

30 1 kg. of ground cellulose is dispersed in 1000 cm.<sup>3</sup> of water, together with 10 g. of  $\alpha,\beta$ -di(5-methylbenzimidazyl-2)-ethylene (cf. Formula 1). By strongly stirring the whole mass is kept in suspension for 30 minutes at a temperature of 50-100° C. After this treatment the fluorescing mass is sucked off and further treated as given in Example 2.

A similar result is attained when on carrying out the process of the present example, the  $\alpha,\beta$ -di(5-methylbenzimidazyl-2)-ethylene is replaced by a same amount of  $\alpha,\beta$ -di(benzimidazyl-2)-ethylene (cf. Formula 11) or  $\alpha,\beta$ -di(5 - methylbenzoxazolyl-2)-ethylene (cf. Formula 12).

## Example 8

45 1 kg. of an ureaformaldehyde resin, prepared according to the method indicated in Example 1 or 2 of the Belgian specification 451,470 is dispersed in 3000 cm.<sup>3</sup> of water together with 10 g. of  $\alpha,\beta$ -di(5-methylbenzimidazyl-2)-ethylene (cf. Formula 1). By strongly stirring, the whole mass is kept in suspension for 30 minutes at a temperature of 50-70° C. After this treatment, the fluorescing mass is sucked off. 50 g. of the strongly fluorescing paste thus obtained are added to 1 kg. of a photographic silver halide emulsion coated on a paper support. The whiteness of the surface color of the photographic paper thus obtained is not lost on rinsing and the photographic element yields after exposure and complete finishing a photographic image wherein the white areas are strongly brightened.

## Example 9

65 1 kg. of an ureaformaldehyde resin prepared according to the method indicated in Example 1 or 2 of the Belgian specification 451,470 is suspended in 3000 cm.<sup>3</sup> of water. To this suspension are added 1000 cm.<sup>3</sup> of a 1% ethanol solution of the compound 4,5-diphenylimidazolone-2 (cf. Formula 10). By strongly stirring, the whole mass is kept in suspension for 30 minutes at a temperature of 50-70° C. After this treatment, the fluorescing mass is sucked off and further treated as indicated in Example 8.

The following is a list of the structural formulae of the optical bleaching agents mentioned in the above examples, the numbers of the list corresponding to those set forth

in parentheses following the name of the compound for ease of correlation:

(1)



(2)



(3)



(4)



(5)



(6)



(7)



(8)



(9)



(10)



(11)

5



(12)



The preparation of compounds in the above list are described in the following citations, the initial once again corresponding to the numbers of the structural formulae and examples:

(1) Chem. Abs., B 44 (1950), p. 2251.  
 (2) U.S. patent specification No. 2,600,080.  
 (3) British patent specification 495,479, p. 3, No. 13; German patent specification 752,677, page 8; Danish patent specification No. 63,688 (1945); German patent specification 972,067.

(4) British specification 624,051.  
 (5) F. Benber: Ber., 19 (1886), page 3235.  
 (6) Prepared analogously to British specification No. 624,051.

(7) Id.  
 (8) "Blancophor R" trademark transferred from I. G. Farbenindustrie Aktiengesellschaft to Farbenfabriken Bayer A.G., Danish patent specification 63,688 (1945), German patent specification 972,067, "Zeitschrift für die Erzeugung von Holtzstoff, Zellstoff, Papier und Pappe," Chemische Technologie der Cellulose, 8. Jahrgang, Darmstadt, April 1954, Heft 7/8, A. E. Siegrist "Die Anwendung optischer Aufhellmittel in der Papierindustrie," S. 114-115.

(9) Neunhofer and Rosahl: Chem. Ber., 86 (1953); S. 1146.

(10) Org. Synth. Coll., vol. II, p. 231.  
 We claim:

40. 1. Light-sensitive photographic paper comprising a paper base, a white pigmented coating and a light-sensitive silver halide emulsion layer, said white pigmented coating containing a fluorescent mass comprising a member selected from the group consisting of  $\alpha,\beta$ -di(5-methyl-

benzimidazyl-2)-ethylene,  $\alpha,\beta$ -di(benzimidazyl-2)-ethylene,  $\alpha,\beta$ -di(5-methylbenzoxazolyl-2)-ethylene and 1,3-dioxo-2-butyl-6-acetylamo - 1,2,3H - benz [de] isoquinoline, and a finely divided polyethyleneglycolphthalate.

65. 2. A photographic paper as defined in claim 1, wherein the phthalate is the terephthalate.

3. A photographic paper as defined in claim 1, wherein the phthalate is isophthalate.

4. A photographic paper as defined in claim 1, wherein 70 said polyethylene glycolphthalate contains equal amounts of the moieties of isophthalic acid and terephthalic acid.

5. A photographic paper as defined in claim 1, wherein 75 said polyethylene glycolphthalate contains equal amounts of the moieties of isophthalic acid and *p*-carboxyphenylsulphonic acid.

6. A photographic paper as defined in claim 1, wherein the fluorescent agent is alpha,beta-di(5-methylbenzimidazyl-2)-ethylene.

7. A photographic paper as defined in claim 1, wherein the fluorescent agent is alpha,beta-di-(benzimidazyl-2)-ethylene. 5

8. A photographic paper as defined in claim 1, wherein the fluorescent agent is alpha,beta-di(5-methyl-benzoxazolyl-2)-ethylene.

9. A photographic paper as defined in claim 1, wherein 10

the fluorescent agent is 1,3-dioxo-2-butyl-6-acetylaminol,2,3H-benz [de] isoquinoline.

References Cited in the file of this patent

UNITED STATES PATENTS

2,723,197 Libby et al. ----- Nov. 8, 1955

FOREIGN PATENTS

878,823 France ----- Nov. 2, 1942

58,372 Holland ----- Oct. 15, 1946